

## UNITED STATES PATENT OFFICE

2,112,576

## PREPARATION OF CELLULOSE XANTHATE SOLUTIONS

George A. Richter, Berlin, N. H., assignor to Brown Company, Berlin, N. H., a corporation of Maine

No Drawing. Application March 1, 1937,  
Serial No. 128,492

6 Claims. (Cl. 260—100)

In preparing cellulose xanthate solutions or viscose for conversion into artificial silk, films, and other ultimate products, it has been the practice to soak sheets of cellulose, such as bleached sulphite pulp, with caustic soda solution of about 18% strength, squeeze excess solution from the sheets, comminute the sheets into crumbs of so-called soda cellulose, age the crumbs under controlled temperature for a considerable period of time, expose the aged crumbs to carbon bisulphide vapors in a rotating drum, and to dissolve the resulting cellulose xanthate in water of the appropriate alkalinity. The plant space, equipment, and labor costs for performing the various steps of such a process are quite expensive; and, moreover, it takes days before the wood pulp used as raw material is transformed into a cellulose xanthate solution or viscose of the desired quality.

I have conducted extensive research on the preparation of cellulose xanthate solutions with a view toward accomplishing in a single operation or step the transformation of cellulose fiber into a cellulose xanthate solution or viscose of quality suitable for such purposes as manufacturing artificial silk, films, etc., and thus reducing materially the plant space, equipment, labor costs, and time heretofore required in so doing. As can readily be appreciated, the success of such research depended upon the realization of cellulose xanthate solution or viscose substantially free from residual or unxanthated cellulose and capable of yielding artificial silk, films, etc., of substantially as good physical and chemical properties as the same ultimate products derived from cellulose xanthate solution as heretofore prepared.

As disclosed in my application Serial No. 37,-043, filed August 20, 1935, I have found that one factor contributing very importantly to the success of a one-step xanthating process is the viscosity of the cellulose fiber used as raw material and that it is only when the fiber is of a solution viscosity less than 1 and preferably from 0.2 to 0.4 that it reacts smoothly and substantially completely in a single mixing operation with the caustic soda solution and carbon bisulphide calculated to yield viscose of the desired cellulose content and causticity, for instance, a cellulose and caustic soda content of about 6% to 10% each. I have now found that while solution viscosity of the fiber is a very important criterion of the suitability of the cellulose fiber for a one-step xanthating operation, there is another factor that controls the suitability of the fiber for such purpose, namely, the beta cellulose content of the fiber and that unless the beta cellulose content of the fiber falls within a certain range, the fiber may not be satisfactorily xanthatable into a viscose syrup by the one-step xanthating op-

eration even when it is possessed of the requisite low solution viscosity. To be sure, the fiber should have an appropriately high alpha cellulose content in order to yield viscose of suitable quality, particularly for such purposes as rayon and film manufacture, but it came as a distinct surprise to me that the beta cellulose content of the fiber also importantly influences the one-step xanthating reaction and further that in order to arrive at consistently satisfactory viscose by the one-step xanthating operation the beta cellulose content of the fiber must fall within a certain range higher than that of the pulps heretofore used as raw material for viscose-making. In accordance with the present invention, therefore, I use as raw material for a one-step xanthating operation wood pulp or other cellulose fiber which not only possesses an appropriate alpha cellulose content and appropriately low solution viscosity but whose beta cellulose content falls outside the beta cellulose content range of the wood pulps generally used heretofore in the usual process of viscose-making.

The industry devoted to usual viscose-rayon manufacture has heretofore generally employed as raw material bleached sulphite wood pulp having the following characteristics:

|                         |            |
|-------------------------|------------|
| Alpha cellulose content | 88 to 89%  |
| Beta cellulose content  | 3 to 5%    |
| Gamma cellulose content | 4 to 8% 30 |
| Viscosity               | 3.0 to 6.0 |

Some of the beta cellulose and most of the gamma cellulose components of such pulp are extracted or dissolved to an appreciable extent when the sheeted pulp undergoes soaking in strong caustic soda solution as accomplished in the usual viscose-rayon process; and this extraction is desirable by reason of the fact that the gamma cellulose appears as undesirable or degraded forms of cellulose in the viscose solution and thus detracts from the quality of the rayon produced from the viscose. In contradistinction to such pulp used in the usual viscose-rayon process, the pulp entering into the one-step xanthating process hereof is characterized by lower gamma cellulose content but higher beta cellulose content. In other words, the present invention can be regarded as involving the use as raw material of a pulp wherein the gamma cellulose content of the usual pulp is replaced to a large extent by beta cellulose which, when kept within a certain range, does not detract significantly from the strength and other qualities of the rayon producible from the pulp while at the same time promoting the desired one-step xanthating reaction on the pulp.

The cellulose fiber for the purposes hereof may be produced from cellulose fibers of various origins, for instance, bleached sulphite, bleached kraft, or other bleached chemical wood pulps,

cotton, cotton linters, etc. Indeed, the bleached sulphite pulp ordinarily used for viscose-making may be chemically processed to acquire the characteristics of the pulp suitable for the one-step xanthating reaction hereof. Thus, ordinary bleached sulphite pulp having the characteristics hereinbefore given may be treated at a consistency of about 4% to 10% with a solution of caustic soda of upwards of about 6% strength containing the appropriate amount of an oxidant, for instance, about 8% to 15% sodium hypochlorite, based on the dry weight of fiber. The particular amount of sodium hypochlorite or other oxidant employed depends in large measure upon the solution viscosity of the starting pulp; and in any event sufficient oxidant is used to cause a reduction of the solution viscosity of the pulp to a value below 1, preferably distinctly below 1, as hereinafter noted. The treatment of the pulp with the solution may be carried out at a temperature of about 35° to 45° C. for a period of about two to four hours, whereupon the pulp may be washed. A typical washed product resulting from the foregoing processing has the following characteristics.

|                         |      |
|-------------------------|------|
| Alpha cellulose content | 90%  |
| Beta cellulose content  | 8%   |
| Gamma cellulose content | 2%   |
| Viscosity               | 0.35 |

Such a pulp product is eminently suitable for the one-step xanthating process hereof.

It is possible to vary the conditions under which bleached sulphite or other chemical wood pulp is processed to produce the pulp product required for the purposes hereof. Thus, the caustic soda solution may be of 6% to 11% or greater strength and, as already indicated, may contain various amounts of oxidant, depending upon the viscosity of the original pulp. Such a solution may be applied to the pulp at temperatures ranging from 30° to 60° C., within which temperature range it is possible to increase the beta cellulose content of the pulp so that its percentage falls within the range desired in the finished pulp while decreasing the gamma cellulose content of the pulp to the appropriately low value and/or keeping it at such value. In any particular case, the various conditions under which the pulp is processed are so correlated as to result in a finished pulp product having the following characteristics:

|                                             |           |
|---------------------------------------------|-----------|
| Alpha cellulose content                     | 87 to 93% |
| Beta cellulose content                      | 6 to 12%  |
| Gamma cellulose content                     | 1 to 3%   |
| Viscosity preferably distinctly less than 1 |           |

The alpha and beta cellulose contents of such a finished pulp product are very significant. Thus, when the alpha cellulose content of a pulp is appreciably greater than 93%, it is generally difficult to convert such pulp by a one-step xanthating reaction into cellulose xanthate solution of the desired filterability and freedom from unxanthated or residual cellulose or gelatinous cellulose particles. It is evidently the case that the beta cellulose content of the finished pulp product hereof is readily and completely xanthatable and induces ready and complete xanthation of the alpha cellulose content of the pulp in a one-step xanthating reaction. Although the role played in the xanthating reaction by the beta cellulose of such a pulp is not fully understood, it may be the case that the xanthating reagents, as they react quickly on the substantial amount

of beta cellulose occurring in and throughout the fiber wall or structure, are brought immediately into contact with more fiber surface throughout the fiber wall and, because of the resulting intimacy or large surface of contact with the alpha cellulose content of the fiber, react on the alpha cellulose more vigorously than is otherwise the case. As already indicated, the xanthation of cellulose pulp containing gamma cellulose means that the gamma cellulose appears as undesirable degraded cellulose in the viscose; and since in the one-step xanthating process hereof the gamma cellulose content of pulp is not partially extracted with caustic soda solution as in the usual viscose-rayon process but is completely xanthated, the gamma cellulose content of the pulp hereof must be kept at a minimum in order to enable the preparation of satisfactory viscose therefrom. Indeed, if the alpha cellulose content of the pulp hereinbefore described is permitted to fall to a value much below 87% with a corresponding rise in its gamma cellulose content, the pulp, although readily xanthatable to completion in a one-step xanthating reaction, is unsuitable for viscose-making by reason of the fact that the rayon producible therefrom is lacking in requisite strength and other qualities.

The one-step xanthating reaction on the pulp used herein as raw material for viscose-making may be conducted as disclosed in my application Serial No. 37,043, filed August 20, 1935, according to which the pulp hereof is admixed with water, caustic soda, and liquid carbon bisulphide in proportions calculated to lead directly to a cellulose xanthate solution of about 6% to 10% cellulose and caustic soda content each. In some instances, the pulp may advantageously be sheeted on a papermaking or board-forming machine and the sheets or boards then reduced to small pieces or chips for the one-step xanthating operation, as disclosed in my application Serial No. 58,539, filed January 10, 1936. According to such latter application, the pieces or chips of interfeited pulp fibers are first soaked with caustic soda solution of mercerizing strength so as to soften and swell them, whereupon the pieces or chips may be disintegrated in the presence of diluting water into a fiber suspension substantially devoid of fiber aggregates and the suspension, whose causticity and fiber content has preferably been controlled during initial soaking and dilution to yield a finished xanthate solution of a cellulose and caustic soda content each falling within the range of 6% to 10%, is then treated with carbon bisulphide and mixed therewith until the ingredients have reacted substantially to completion to yield the desired cellulose xanthate solution.

A procedure embodying the present invention and involving the use of pulp in chip form, the xanthation of the defiberized chips in the presence of caustic soda and water in amount corresponding to a caustic soda solution of greater than 10% strength, and the dilution of the resulting viscose or cellulose xanthate solution with water to the desired final cellulose and caustic soda contents may be carried out substantially as follows. The pulp chips, which may consist of pulp having an alpha cellulose content of 90%, a beta cellulose content of 8%, a gamma cellulose content of 2%, and a solution viscosity of, say, 0.3, may be wetted with 16% caustic soda solution at 20° C. in sufficient volume to provide wetted chips wherein the dry cellulose to caustic soda ratio is 7.6. The volume of 16% caustic soda

solution necessary for this purpose ensures, upon thorough defiberization or disintegration of the solution-impregnated chips, a thick or salve-like mass practically devoid of free or unabSORBED 5 solution. The wetted chips may then be thoroughly defiberized or disintegrated at 20° C., preferably in mixing and tumbling apparatus of the type disclosed in application Serial No. 53,689, filed December 10, 1935, so as to produce the thick 10 or salve-like mass, which defiberizing or disintegrating operation may require about fifteen minutes in such apparatus. To the resulting thick mass of cellulose fiber and caustic soda solution may then be added liquid carbon bisulphide in 15 the amount of about 33% and pine oil in the amount of about 0.01%, based on the weight of dry cellulose. The pine oil tends to react with the caustic soda to form a soapy emulsifying agent which promotes microscopically fine particle size 20 emulsification of the carbon bisulphide in the caustic soda solution and more rapid and complete xanthation of the cellulose, as disclosed more particularly in application Serial No. 63,876, filed February 14, 1936. Upon operating the mixing 25 blades of the apparatus and tumbling the apparatus as described in application Serial No. 53,689 for a further period of about three hours with the charge of the reacting ingredients at about 20° C., it is found at the end of such period 30 that the ingredients have yielded a thick viscose or cellulose xanthate solution substantially free from residual fiber or gelatinous particles and containing about 14% cellulose, based on the weight of viscose. Water may then be added to 35 the apparatus with its mixing blades in operation in amount to dilute the viscose to the desired final cellulose content, say, 7.4%, based on the weight of the finished viscose, at which cellulose content, the resulting viscose has a caustic soda 40 content of 6.7%, based on the weight of viscose. Such a finished viscose is typical in its cellulose and caustic soda contents of those desired for rayon manufacture. It is to be understood that 45 xanthation may be effected hereby in the presence of water and caustic soda in amounts to correspond to caustic soda solution of greater than 16% strength, say, 18% to 20%, or even greater strength, whereupon the resulting viscose or cellulose xanthation solution may be diluted to the desired final cellulose content and 50 causticity. However, it is usually desirable to use herein, as already indicated, caustic soda solution of such strength and in such volume for the impregnation of the cellulose fiber or chips as 55 to make possible easy and uniform impregnation of the fiber with the caustic soda and the direct xanthation of the resulting mixture, that is, without need of excess caustic soda solution and hence without need of removing excess solution 60 from the mass prior to xanthation.

The process hereof admits of considerable variation particularly in respect to such factors as the causticity and cellulose contents of the xanthate solution prepared thereby, of the temperature conditions under which the xanthation is performed, and of the temperature conditions and causticity of the solution initially employed in preparing the thick or salve-like pulp suspension to which the liquid carbon bisulphide is 65 added. Thus, while a finished viscose syrup of a causticity and cellulose content of about 7% each has been cited as being conventional and desirable for artificial silk and film manufacture, yet it is possible to produce finished viscose solutions by the process hereof of much lower or 70

higher causticity and/or cellulose content. Again, the xanthating reaction has been described as preferably being conducted at about 15° to 20° C. (i. e. ordinary temperatures) so as to dispense with the need and expense of any great refrigeration or cooling, but it is possible and, in some cases may be preferable, to carry out the xanthating reaction at much lower than room temperatures, say, temperatures ranging from slightly above the freezing point to room temperature. In those instances when the xanthating reaction is performed at appreciably lower than room temperature, it has been observed that viscose solutions of excellent clarity are realized, although the mixing of the ingredients requires more power by reason of the markedly higher viscosity of the reacting mixture at such temperatures. The initial soaking or treatment of the pulp with caustic soda solution to form the thick or salve-like suspension subjected to xanthation 10 may also be performed at distinctly sub-room temperatures down to the freezing point and with caustic soda solutions of varying causticity, depending upon the causticity to be realized in the finished xanthate solution. In other words, the causticity of the solution initially employed should be sufficiently great so as to enable the realization of a xanthate solution which directly after the xanthating reaction or upon subsequent dilution with water has the desired causticity in 15 combination with the desired cellulose content. It is thus seen that the present invention although tied down to the use of a pulp of particular combined chemical characteristics in a one-step xanthating process, nevertheless lends itself to considerable variation in so far as concerns the various conditions such as temperature, causticity, cellulose content, carbon bisulphide usage, etc. under which xanthation is effected. The pulp or fiber thus used may be of various origins 20 and in various physical conditions. Thus, the pulp may be derived from hardwoods, such as birch or maple, or from softwoods, such as spruce and fir. Again, the pulp may be used with its fibers in substantially unreduced or uncut condition or it may be broken down into fiber fragments or even powdered cellulose by suitable mechanical treatment prior to subjecting it to the 25 one-step xanthating process hereof.

I wish again to stress the fact that the pulp used for the purposes hereof should have an alpha cellulose content of upwards of about 87%, for, when its alpha cellulose content is very much below such value, viscose prepared therefrom by the one-step xanthating process does 30 not yield rayon or films of satisfactory quality. That the relatively high beta cellulose content in the pulp used herein must be associated with an alpha cellulose content in the pulp of not less than 87% may better be understood from the fact that should cotton or wood pulp be subjected to an acid-hydrolyzing treatment serving to reduce alpha cellulose content in the fiber to, say, 75% or 70% and to raise beta cellulose content to upwards of, say, 10%, the resulting 35 cellulose fiber, although lending itself to quick and complete conversion into viscose by the one-step xanthating reaction, yields as a result of such reaction a viscose quite unsatisfactory for rayon and film manufacture. The point is, as 40 already indicated, that whereas in the usual viscose-making process a substantial proportion of the non-alpha cellulose components in the pulp are removed by extraction in the excess strong caustic soda solution used for preparing soda 45 50 55 60 65 70 75

cellulose, such components remain in the mixture of reacting ingredients in a one-step xanthating process. Accordingly, when hydrolyzed fiber of the composition just cited serves as raw material in a one-step xanthating process, the resulting viscose is so greatly contaminated by degraded celluloses that the rayon, films, or other regenerated cellulose products manufactured therefrom are of unsatisfactory physical and chemical qualities.

Another very important property of the pulp hereinbefore described used for the purposes hereof is the excellent filterability of viscose prepared therefrom by the one-step xanthating process hereof. I have found that unless viscose syrup has a filterability of at least 300 cubic centimeters, as determined by a test hereinafter given, it is not suitable for such practical purposes as the manufacture of rayon. The pulp used for the purpose hereof answers this requirement admirably, as viscose syrup prepared therefrom by the one-step xanthating process hereof has a filterability of at least 500 cubic centimeters.

I shall now give the method used herein for determining the filterability of viscose solution.

#### Viscose samples

These samples contain normally 7.40% cellulose, 6.70% NaOH and 2.25% sulphur. The samples are held idle at 20° C. for 24 hours after their production, before determining their filterability. This permits the escape of air that has become entrained in the viscose during its preparation. The amount held is no greater than the capacity of the filter chamber. In filling the chamber the entire amount is poured and scraped out of the container into the chamber. The samples are not pre-strained through a sieve before using them for this determination of filterability.

#### Filter chamber

This chamber is a pipe having an internal cross-section of 7.0 square inches and an overall length between its two flanged ends of 48 inches. It is mounted in a vertical position. It is covered with a disc on its top, with a perforated rubber gasket between this disc and the top flanged end. This disc is bolted on after an orifice plate, the filter pad, a support, and a discharge pipe have been attached to the lower flanged end, and the viscose sample added to the chamber. The viscose sample may be insufficient to fill the chamber. If it does fill the chamber, its weight is a maximum of only two pounds to the square inch at the filter pad. The top disc carries a pipe connection to a supply of compressed air through an air separator and reducing valve. This valve is set to give an air pressure of 70 pounds on the sample of viscose. The air to the reducing valve is always at a pressure greater than 70 pounds.

The chamber is surrounded by a second pipe to give a 1/2" water jacket. This jacket is welded to the inner faces of the two flanged ends of the unit. A stream of water is circulated up through the jacket from a header supplied by both cold and warm water services. A thermometer pocket is built into this header. The water to the jacket is held at 20° C. by manual control of the water services as read by a thermometer in the pocket. The discharged water is wasted into a drain.

#### Orifice plate

An orifice plate is placed next to the lower flanged end of the filter chamber. These flanged ends have machined-smoothed surfaces. A rub-

ber gasket is placed between the lower flanged end and this orifice plate. It has an opening considerably greater than that of the orifice plate. The orifice plate is a metal disc in which there is a smooth circular opening of exactly one square inch area, in its center. This orifice plate is made of corrosion-resisting material and the area of its opening is checked frequently to assure permanence of the same. The orifice plate is of  $\frac{1}{16}$ " stock to protect it against deformation in its plane surface when bolting the plate, filter pad, support and discharge pipe to the lower flanged end of the filter chamber. The orifice plate has an external circular size which equals that of the circle that is circumscribed with only a little clearance within the bolt circle of the lower flanged end of the filter chamber.

#### Filter pad

The filter pad is a combination of four sheets of cotton fabric popularly called airplane cloth. This fabric is unbleached. The thread count per square inch is 130 x 142,—warp x woof. It weighs 3 ounces per square yard. It has a thickness of 0.006 inch. In making a pad, the sheets are cut each to a size of four inches on a square side and in the two respective directions of its component threads. This filter pad is placed against the lower side of the orifice plate without another inserted gasket present. In finally bolting all the parts to the lower flanged end of the filter chamber, the orifice is seated firmly over this filter pad and thereby there is exposed to the passage of the viscose sample only one square inch area of this filter pad to filter the viscose.

#### Support

To support the filter pad with additional firmness against the orifice and further to prevent its sagging and so a distortion of its area and texture in the surface that is exposed as a filtering medium against the passage of the viscose, there is placed under the pad two metal parts. The first is a piece of woven wire corduroy cloth, 12 x 64 mesh, of Monel metal material, four inches on a square side. This wire corduroy cloth is in turn supported by the second of these metal parts. This is a coarse metallic grid of corrosion-resisting steel about  $\frac{1}{8}$  inch in thickness, perforated with quarter-inch holes spaced as closely together as can be done mechanically. The perforations are all in an area of two inches diameter and these lay under both the orifice opening and adequately beyond its edge. The grid has an outside circular size equalling that of the orifice plate.

#### Discharge pipe

This is a  $\frac{1}{8}$  inch I. D. pipe connection to the opened apex of an inverted cone which extends down from a flange whose size and bolt circle equals that of the lower flanged end of the filter chamber. This flange and the two flanged ends of the filter chamber are each of  $\frac{3}{4}$  inch thickness to prevent their distortion when bolting the parts together. This discharge pipe is placed below the perforated grid support, and when the orifice, filter pad, and two supports are aligned, it is bolted to the flanged end of the filter chamber, with mechanical care used to apply equal firmness around the bolt circle.

#### Operation of a determination of filterability

The open filter chamber, first, has been scrubbed with an oversize, round, coarse brush and rinsed clean and drained. The orifice plate,

filter pad, supports and discharge pipe are assembled and bolted on to the lower end of the filter chamber. The jacket water is adjusted to 20° C. and flowed to temper the assembled filter 5 to 20° C. The 20° C. viscose is poured carefully and slowly into the chamber and the top disc bolted on. Air pressure at 70 pounds is applied. At the first moment of discharge of filtrate, an interval clock is started. The filtrate is received 10 into a calibrated glass receptacle, and the accumulations in cc. are read periodically. The discharged cc. are plotted continuously as abscissae against total time as ordinates. When the curve shows that the rate of discharge of the filtrate 15 approaches zero in relation to elapsed time, then the pad is known to be plugged. An interval of several minutes will have occurred in which no filtrate is discharged. The total cc. of filtrate discharged is the measure of filterability of the 20 viscose.

Always there is used a new filter pad for each determination, and the orifice plate, gaskets, supports and discharge pipe are always freshly washed and dried before use. The woven corduroy 25 cloth is blown dry with compressed air and inspected to assure that none of the mesh openings are closed.

*Quality standard of filterability*

30 I have determined that for the satisfactory manufacture of rayon from viscose, a sample of the viscose tested by the foregoing method should deliver a total of at least 500 cubic centimeters of filtrate.

35 The solution usually employed as a standard for measuring the viscosity of cellulose pulp is a cuprammonium cellulose solution of prescribed cellulose concentration, the viscosity being determined by measuring the time of efflux of a definite

40 volume of such solution under standard conditions, through an orifice of standard size. The solution viscosity of fiber is hereinbefore given in absolute C. G. S. units or poises, and is determined by measuring the viscosity of a solution of

45 6 grams of fiber in a cuprammonium solution composed of 225 cc. of 28% ammonia water containing 9 grams of so-called "copper hydrate" powder. This "copper hydrate" powder is in reality a basic copper nitrate. The C. G. S. unit

50 is employed because it is definite, denoting a viscosity 100 times that of water at 20° C., wherefore, a cuprammonium cellulose solution of standard composition identifying a fiber as having a solution viscosity of 10 is 1000 times as viscous as

55 water at 20° C. The method of determining or measuring solution viscosity of cellulose fiber used herein is that described by me in much greater detail in "Industrial and Engineering Chemistry", volume 23, page 136, 1931; and inasmuch as the

60 description of my viscosity-testing method as given in that publication affords the particular criterion or test used herein, it is to be understood that my reference to such description is intended to incorporate such description as a part

65 hereof. Since the methods of determining alpha-, beta-, and gamma-cellulose used for the purpose of the invention hereof are also set forth in detail on pages 134 and 135 of the publication just mentioned, it is to be further understood that the description of such methods as given in that publication are intended to be made part hereof.

I claim:

1. A process of producing viscose, which comprises treating cellulose fiber of the nature of chemical wood pulp and cotton with caustic soda solution containing an oxidant under conditions of caustic soda and oxidant concentration, temperature, and time to yield a fiber having an alpha cellulose content of about 87 to 93%, a beta cellulose content of about 6 to 12%, and a viscosity less than 1; washing the fiber substantially free of such treating solution; and mixing the fiber 10 with caustic soda solution and liquid carbon bisulphide in amount to xanthate the fiber substantially completely and to form viscose.

2. A process of producing viscose, which comprises treating bleached chemical wood pulp at 15 about 30° to 60° C. with caustic soda solution of a strength upwards of about 6% and containing oxidant in sufficient amount to cause a reduction of the solution viscosity of the pulp to a value below 1; continuing the treatment for a sufficient 20 period of time to yield a pulp product having an alpha cellulose content of about 87 to 93%; a beta cellulose content of about 6 to 12%, and a viscosity less than 1; washing the pulp product substantially free of such treating solution; and mixing the resulting pulp product with caustic soda solution and liquid carbon bisulphide in amount to xanthate the fiber substantially 25 completely and to form viscose.

3. A process of forming viscose in one step, 30 which comprises commingling caustic soda solution and liquid carbon bisulphide with cellulose fiber having an alpha cellulose content of about 87 to 93%, a beta cellulose content of about 6 to 12%, and a solution viscosity less than 1, the caus- 35 ticity of said solution and its proportion relative to the fiber being controlled to yield viscose of a caustic soda and cellulose content of about 6% to 10% each.

4. Cellulose fiber capable of being substantial- 40 ly completely xanthated and dissolved to form viscose by direct admixture with caustic soda solution and liquid carbon bisulphide, said fiber having the following characteristics:

Alpha cellulose content..... 87 to 93% 45  
Beta cellulose content..... 6 to 12%  
Viscosity less than 1

5. Cellulose fiber capable of being substantial- 50 ly completely xanthated and dissolved to form viscose by direct admixture with caustic soda solution and liquid carbon bisulphide, said fiber having the following characteristics:

Alpha cellulose content..... 87 to 93% 55  
Beta cellulose content..... 6 to 12%  
Gamma cellulose content..... 1 to 3%  
Viscosity less than 1

6. A soda-cellulose mixture capable of being substantially completely xanthated by direct ad- 60 mixture therewith of liquid carbon bisulphide and containing such proportions of cellulose and caustic soda solution as to yield upon such xanthation viscose of at least 6% cellulose and caustic soda contents each, the cellulose in said soda-cellulose 65 mixture having the following characteristics:

Alpha cellulose content..... 87 to 93%  
Beta cellulose content..... 6 to 12%  
Viscosity less than 1

GEORGE A. RICHTER.